# EUROPEAN PATENT SPECIFICATION

(11) **EP 2 083 973 B1**
(45) Date of publication and mention of the grant of the patent: **17.08.2011**
(21) Application number: 07853890.7
(22) Date of filing: 10.10.2007
(51) Int. Cl.: B26F 1/26, D04H 1/54

(54) **APERTURED NONWOVEN FABRIC AND PROCESS AND APPARATUS FOR PRODUCING SAME**
VLIESSTOFF MIT ÖFFNUNGEN UND HERSTELLUNGSVERFAHREN UND -VORRICHTUNG DAFÜR
Tissu non-tissé perforé, et procédé et appareil de fabrication associés

(30) Priority: 17.10.2006 US 829778 P
(43) Date of publication of application: 05.08.2009
(73) Proprietor: Fiberweb Simpsonville, Inc., Simpsonville SC 29681 (US)
(72) Inventor: BAER, Samuel Charles, Greenville, SC 29615 (US); GILLESPIE, Jay Darrell, Simpsonville, SC 29681 (US); NEWKIRK, David D., Greer, SC 29650 (US)
(74) Representative: Noel, Chantal Odile
(86) International application number: PCT/US2007/080901
(87) International publication number: WO 2008/048829

(56) References cited:
- EP-A- 0 620 087
- WO-A-2004/087384
- DE-U1-202004 009 078
- US-A- 5 188 625

## Description

### FIELD AND BACKGROUND OF THE INVENTION

This invention relates to apertured nonwoven fabrics and to a method and apparatus for producing such fabrics.

It is desired to produce a fabric that has a total open area greater than about 10% of the fabric's surface at a line speed that is typical of commercial nonwoven textile production lines. This will allow production of a perforated fabric on the fabric manufacturing line and thus not require a costly separate manufacturing step. If the fabric is comprised of thermoplastic fibers then the aperturing can be accomplished continuously through a combination of heat and pressure applied at selected points on the fabric.

Several processes to produce large apertures in thermoplastic fabrics are described in the patent literature. Shimalla in US Patent No. 4,588,630 describes a two-step process where a high pressure thermal embossing calender melts small holes into a thermoplastic fabric and the fabric is then subjected to non-recoverable stretch in the MD and/or CD directions to enlarge the holes. The melted edges of eth perforation may contribute to the strength and integrity of the apertured fabric.

Benson in US Patent No. 5,916,661 describes an alternate two-step process where a point bonded fabric is subjected to a second thermal emboss step where selected points on the fabric are weakened via melting but are not actually perforated. The selectively weakened fabric in then subjected to an incremental stretching process than causes the weakened points to first rupture into narrow holes and them expend to form large open apertures in the fabric.

Both the Shimalla and Benson patents have a key common feature of requiring a high degree of non-recoverable stretching of the thermally perforated or thermally weakened fabric to significantly enlarge the initial small apertures or weakened regions of the pre-stretched fabric.

Coslett et al. in US patent Nos. 5,656,119; 5,567,501 and 5,830,555 describe thermoplastic fabric and fabric/film laminates that are optimum for forming apertures where each perforation roll emboss point has a contact area with the fabric that is essentially the same dimension as the resulting aperture. The patents teach that a blend of higher melting fiber with either lower melting temperature fibers or film favor clean, well-defined apertures. Low elongation, high tenacity polypropylene staple fibers were preferred over higher elongation lower tenacity polypropylene fibers and were superior in forming well defined apertures. Gillespie et al. in US Patent No. 6,632,504 also identifies fabric fiber compositions that yield fabrics that are especially amenable to thermal aperturing via thermal embossing followed by significant stretching.

There is a need for a process that allows fabric perforation at commercial nonwoven line production speeds while yielding a perforation pattern that is a precise replication of the desired fabric design. The Shimalla and Benson processes require extensive fabric distortion via MD and/or CD stretching to achieve larger apertures. The Coslett et al. process can yield large apertures but the thermal and compressive energies that perforate the fabric are distributed over the full area of the resulting perforation which can severely limit the maximum line speed that clean apertures can occur.

### SUMMARY OF THE INVENTION

In one aspect, the present invention provides a nonwoven fabric comprised of thermoplastic fibers bonded to one another at a multiplicity of bond sites to form a coherent, strong nonwoven web, and a plurality of apertures formed in the nonwoven fabric by removal of selected portions of the nonwoven web, the apertures forming an open area of at least 10 percent of the fabric surface area. A chad formed from the removed portion of nonwoven web may be found releasably attached to at least some of the apertures, and a margin of fused thermoplastic fiber extends along the periphery of the chad. A margin of fused thermoplastic fiber may also extend along the periphery of the apertures. The nonwoven fabric may be of various constructions, including carded thermal bond nonwoven fabrics, airlaid nonwoven fabrics and spunbond nonwoven fabric comprised of continuous filaments of thermoplastic polymer. The apertures are clean-cut and well defined and the fabric has not been subjected to non-recoverable stretching.

The present invention also provides a method of making an apertured nonwoven fabric comprising steps of: directing a nonwoven fabric comprised of thermoplastic fibers along a predetermined path of travel into and through an embossing station; contacting the nonwoven fabric at the embossing station with an embossing roll having a predetermined patterned surface; applying heat and pressure to the nonwoven fabric with the patterned surface to thermally fuse the thermoplastic fibers along a plurality of enclosed paths defining selected areas of the surface of the fabric in which apertures are to be formed; and removing the selected areas of the fabric from the remainder of the fabric. The plurality of enclosed paths of thermally fused fibers may form embossed areas that constitute no more than 10 percent of the fabric surface area and surround areas of the nonwoven fabric in which the thermoplastic fibers are unfused and unembossed. In certain embodiments, the plurality of enclosed paths of thermally fused fibers have a surface area between 2% and 20% of the area circumscribed by the enclosed paths.

The present invention also relates to an embossing roll for producing an apertured nonwoven fabric. The roll comprises a cylindrical body and a plurality of raised embossments at predetermined spaced locations over the cylindrical surface of the body, with the raised embossments including a raised land surface for contacting the fabric extending along a closed path along the periphery of the raised embossment, and a recessed surface surrounded by the raised land surface, and wherein the raised land surface has a surface area between 2% and 20% of the area surrounded by the raised land surface. In certain advantageous embodiments, the embossments are present on the roll at a density such that the raised land surface and the surrounded recessed surface constitute at least 10 percent of the surface area of the cylindrical surface.

### BRIEF DESCRIPTION OF THE DRAWINGS

Having thus described the invention in general terms, further aspects of the invention will become apparent from the detailed description which follows, and from the accompanying drawings, in which:
FIG. 1 illustrates one embodiment of a bond pattern design for an embossing roll;
FIG. 2 is a top view of the roll;
FIG. 3a is a schematic illustration of a thermal perforation process;
FIG. 3b is a schematic illustration of an ultrasonic perforation process;
FIG. 4 is a magnified photograph showing a perforated fabric showing apertures with and without chad removal; and
FIG. 5 is a magnified view of a single aperture showing the chad loosely held by the residual fibils along the circumference of the emboss region.

### DETAILED DESCRIPTION

The invention disclosed herein features a 1) emboss pattern design where the individual bond points are concave in design so that only the outer peripheral edge of each bond point is in contact with the fabric to be apertured in the nip and 2) a post embossing step is employed to clear the fabric apertures of the residual fabric that was inside of the emboss line of each bond point without any non-recoverable stretching of the fabric.

FIG 1 shows one embodiment of such a bond pattern design (A) with a raised annular peripheral edge (B) around a central recess or void area (C). FIG 2 shows the arrangement of the bond points (A) on a patterned embossing calender roll (D). In this embodiment the cumulative surface area occupied by the oval bond points is about 35% of the surface area of the embossing roll and the cumulative surface area of the raised annular edges on each bond point is about 5% of the surface area of the embossing roll. Thus the perforation energy in the nip is concentrated on only about 5% of the surface area of the fabric passing through the nip. This invention is not limited to any particular bond point shape or array of bond points on the embossing roll. In general, a suitable bond point design would have the fabric contact area of the bond point be between 2% and 20% of the area circumscribed by the total bond point. The size, shape, and number of bond points per unit area would vary according to the requirement of the particular application. The inventors anticipate that this method of continuous fabric perforation would have greatest utility where the desired open area of the fabric is greater than 10% of the fabric surface.

The localized heating at the fabric contact points can be either driven by thermal conduction from a heated calender roll or by high-frequency vibration of an ultrasonic horn.

The bond point shown in FIG 1 is designed to melt away the fabric at the contact point leaving a chad of fabric that drops out of the aperture. We found the surprising result that under proper raw material selection and embossing nip settings the chad would be very loosely held in the aperture as the embossed, scored fabric exited the nip. This allows for an easy removal of the chads from their respective apertures by a simple air jet (FIG 3a and 3b) as the fabric moved away from the nip. The chad removal action of the air jet may be assisted or substituted by a set of brush rolls applied to the surface of the embossed, scored fabric.

The observed fabric behavior is preferred over complete chad punch-out in the nip because the chads do not clog up the recessed void spaces of the embossing roll and the chad removal station could be removed from the vicinity of the nip to allow for ease of collection of the chads for potential recycle. It is important to note that non-recoverable stretch of the sort described in Shimalla and Benson was not at all required to remove the nonwoven fabric chads.

FIG. 4 shows a magnified post-emboss fabric where some of the chads have been removed and some of the chads remain in place. FIG 5 shows a close-up view of a chad that is being partially held in place by some of the unsevered fibers of the nonwoven fabric. The fabrics shown in FIGS. 4 and 5 were embossed with the pattern described in FIGS. 1 and 2.

The advantages of this fabric aperturing process over the prior art are several. Large (e.g. 10% or greater) open areas can be created in a suitable fabric at high speed without non-recoverable fabric stretching in any direction. Non-recoverable stretching of the fabric can degrade material properties. The shape and distribution of the individual apertures can be precisely defined and will not be unpredictably distorted by subsequent web stretching. Thus, the apertures can define various patterns in the nonwoven fabric. The energy to achieve the aperture is concentrated only where it is required to cut out the large aperture. This allows for successful web aperturing at the maximum possible line speed.

### EXAMPLE 1

An embossing roll with raised embossments forming a land area of about 5% of the area of the embossing roll was thermally emboss a 18 gram per square meter spunbond polypropylene spunbond nonwoven fabric at a line speed of 305 meters per minute.

### EXAMPLE 2

An embossing roll as illustrated in FIGS. 1 and 2 was designed to produce an open area of at least 20% of the fabric area, but with the an annular raised land surface that would have a fabric contact area of no more than 5%. This embossing roll was used in a calender stand against a plain surfaced anvil roll. The nip pressure was set to 86,25 bar 8.63·10⁶N/m² (1250 psi). The patterned roll was heated to 254°C and the anvil roll at 256°C. Operating at a line speed of 100 feet/minute 30.5 m/minute this calender was employed to thermally emboss a 28.1 gram per square meter spunbond nonwoven fabric formed from continuous filaments of a sheath-core bicomponent structure with a 50% polyethylene sheath and 50% polypropylene core. When a stream of high velocity air was directed against the fabric, the chads were easily blown out of the fabric, leaving clean well-defined apertures without any tearing or distortion of the fabric. The apertured fabric was still soft.

### EXAMPLE 3

The embossing procedure of Example 2 was performed on a nonwoven spunbond fabric in which the filaments had a segmented pie cross-sectional configuration consisting of six segments of alternating polypropylene and polyethylene. Apertures similar to those of Example 2 were observed.

### EXAMPLE 4

An 18 gram per square meter spunbond polypropylene nonwoven fabric was thermally embossed using a embossing procedure similar to Example 2 except that the roll temperatures were increased.

### EXAMPLE 5

The embossing procedure of Example 2 was carried out on a 24.1 gram per square meter spunbond-meltblown-spunbond composite nonwoven fabric laminate. The chads were readily removed by air and/or abrasion. Clean, well-defined apertures were observed and the fabric remained soft.

## Claims

1. A nonwoven fabric comprised of thermoplastic fibers bonded to one another at a multiplicity of bond sites to form a coherent, strong nonwoven web, and a plurality of apertures formed in the nonwoven fabric by removal of selected portions of the nonwoven web, the apertures forming an open area of at least 10 percent of the fabric surface area, the fabric including a chad formed from the removed portion of nonwoven web releasably attached to at least some of the apertures, a margin of fused thermoplastic fiber extending along the periphery of the chad.

2. The fabric of claim 1 including a margin of fused thermoplastic fiber extending along the periphery of the apertures.

3. The fabric of any one of the preceding claims, wherein the nonwoven fabric is selected from the group consisting of carded thermal bond nonwoven fabric comprising thermoplastic staple fibers, an airlaid nonwoven web comprising thermoplastic staple fibers, and a spunbond nonwoven fabric comprised of continuous filaments of thermoplastic polymer.

4. The fabric of any one of the preceding claims in which the fabric is unstretched.

5. A spunbond nonwoven fabric comprised of continuous thermoplastic filaments randomly arranged and bonded to one another at a multiplicity of bond sites to form a coherent, strong spunbond nonwoven web, and a plurality of apertures formed in the nonwoven fabric by removal of selected portions of the nonwoven web, the apertures forming an open area of at least 10 percent of the fabric surface area, the spunbond nonwoven fabric including a chad formed from the removed portion of spunbond nonwoven web releasably attached to at least some of the apertures, a margin of fused thermoplastic fiber extending along the periphery of the chad.

6. A method of making an apertured nonwoven fabric comprising:
- directing a nonwoven fabric comprised of thermoplastic fibers along a predetermined path of travel into and through an embossing station;
- contacting the nonwoven fabric at the embossing station with an embossing roll having a predetermined patterned surface;
- applying heat and pressure to the nonwoven fabric with the patterned surface to thermally fuse the thermoplastic fibers along a plurality of enclosed paths defining selected areas of the surface of the fabric in which apertures are to be formed, forming chads that are releasably attached to some of the apertures, and forming a margin of fused thermoplastic fibers extending around the periphery of the chads; and
- removing said selected areas of the fabric from the remainder of the fabric.

7. The method of claim 6 wherein the selected areas constitute at least 10 percent of the fabric surface area.

8. The method of claim 6 wherein the plurality of enclosed paths of thermally fused fibers form embossed areas that constitute no more than 10 percent of the fabric surface area and surround areas of the nonwoven fabric in which the thermoplastic fibers are unfused and unembossed.

9. The method of claim 8 wherein the plurality of enclosed paths of thermally fused fibers have a surface area between 2% and 20% of the area circumscribed by the enclosed paths.

10. The method of any one of claims 6 to 9 wherein the step of removing said selected areas comprises directing air onto the fabric to remove said selected areas.

11. The method of any one of claims 6 to 9 wherein the step of removing said selected areas comprises contacting the fabric with brushes to remove said selected areas.

12. The method of any one of claims 6 to 11 wherein the step of applying heat and pressure comprises contacting the embossing roll with a heated anvil roll or with an ultrasonic anvil.

13. An embossing roll for producing an apertured nonwoven fabric comprising a cylindrical body and a plurality of raised embossments at predetermined spaced locations over the cylindrical surface of the body, said raised embossments including a raised land surface for contacting the fabric extending along a closed path along the periphery of the raised embossment, and a recessed surface surrounded by the raised land surface, and wherein the raised land surface has a surface area between 2% and 20% of the area surrounded by the raised land surface, the embossments being designed to leave chads that are releasably attached to some of the apertures and to include a margin of fused thermoplastic fiber extending along the periphery of the chads.

14. The roll of claim 13, wherein the embossments are present on the roll at a density such that the raised land surface and the surrounded recessed surface constitute at least 10 percent of the surface area of the cylindrical surface.

15. The roll of claim 13 or 14 wherein the raised land surface constitutes from 2 to 10 percent of the surface area of the area surrounded by the raised land surface

16. The roll of claim 13, 14 or 15 wherein the raised land surface has a width of from 10 to 30 percent of the maximum width of the raised embossment.

17. The roll of any one of claims 13 to 16 wherein the raised embossments have a circular or oval configuration.

## Patentansprüche

1. Vliesstoff, bestehend aus thermoplastischen Fasern, die an einer Vielzahl von Verbindungspunkten unter Bildung eines kohärenten, starken Vliesstoffes aneinander gebunden sind, und einer Vielzahl von Öffnungen, die durch Entfernung von ausgewählten Teilen des Vliesgewebes im Vliesstoff ausgebildet sind, wobei die Öffnungen einen offenen Bereich von wenigstens 10% des Stoffoberflächenbereichs bilden, der Stoff einen Stanzabfall, gebildet aus dem entfernten Teil des Vliesgewebes, an wenigstens einigen der Öffnungen lösbar befestigt umfasst, wobei sich ein Rand aus verschmolzener thermoplastischer Faser entlang der Peripherie des Stanzabfalls erstreckt.

2. Stoff gemäß Anspruch 1, der einen Rand aus verschmolzener thermoplastischer Faser umfasst, cer sich entlang der Peripherie der Öffnungen erstreckt.

3. Stoff gemäß einem der vorangehenden Ansprüche, wobei der Vliesstoff aus der Gruppe, bestehend aus kardiertem, thermisch gebundenem Vliesstoff, der thermoplastische Stapelfasern umfasst; einem luftgelegten Vliesgewebe, das thermoplastische Stapelfasern umfasst, und einem Spinnvlies, das aus kontinuierlichen Filamenten aus thermoplastischem Polymer besteht, ausgewählt ist.

4. Stoff gemäß einem der vorangehenden Ansprüche, wobei der Stoff ungestreckt ist.

5. Spinnvliesstoff, bestehend aus kontinuierlichen thermoplastischen Filamenten, die statistisch angeordnet sind und an einer Vielzahl von Verbindungspunkten unter Bildung eines kohärenten, starken Spinnvliesgewebes aneinander gebunden sind, und einer Vielzahl von Öffnungen, die durch Entfernung von ausgewählten Teilen des Vliesgewebes in dem Vliesstoff ausgebildet sind, wobei die Öffnungen einen offenen Bereich von wenigstens 10% des Stoffoberflächenbereichs bilden, der Spinnvliesstoff einen Stanzabfall, gebildet aus dem entfernten Teil des Spinnvliesgewebes, an wenigstens einigen der Öffnungen lösbar befestigt umfasst, wobei sich ein Rand aus verschmolzener thermoplastischer Faser entlang der Peripherie des Stanzabfalls erstreckt.

6. Verfahren zur Herstellung eines mit Öffnungen versehenen Vliesstoff, umfassend:
- Steuern eines Vliesstoffs, bestehend aus thermoplastischen Fasern, entlang einer vorbestimmten Bewegungsbahn in und durch eine Prägestation;
- Irkontaktbringen des Vliesstoffs an der Prägestation mit einer Prägewalze, die eine vorbestimmte gemusterte Oberfläche hat;
- Anwenden von Wärme und Druck auf den Vliesstoff mit der gemusterten Oberfläche, um die thermoplastischen Fasern entlang einer Vielzahl von geschlossenen Wegen, die ausgewählte Bereiche der Oberfläche des Stoffs definieren, in welchen Öffnungen zu bilden sind, thermisch zu verschmelzen, wodurch Stanzabfälle gebildet werden, die lösbar an einigen der Öffnungen befestigt sind, und wobei ein Rand aus verschmolzenen thermoplastischen Fasern gebildet wird, der sich um die Peripherie der Stanzabfälle erstreckt, und
- Entfernen der ausgewählten Bereiche des Stoffs vom Rest des Stoffs.

7. Verfahren gemäß Anspruch 6, wobei die ausgewählten Bereiche wenigstens 10% des Stoffoberflächenbereichs bilden.

8. Verfahren gemäß Anspruch 6, wobei die Vielzahl von geschlossenen Wegen thermisch verschmolzener Fasern geprägte Bereiche bildet, die nicht mehr als 10% des Stoffoberflächenbereichs bilden und Bereiche des Vliesstoffs umgeben, in denen die thermoplastischen Fasern unverschmolzen und ungeprägt sind.

9. Verfahren gemäß Anspruch 8, wobei die Vielzahl der geschlossenen Wege von thermisch verschmolzenen Fasern einen Oberflächenbereich von zwischen 2% und 20% der Fläche, die von den geschlossenen Wegen umschrieben wird, hat.

10. Verfahren gemäß einen der Ansprüche 6 bis 9, wobei der Schritt des Entfernens der ausgewählten Bereiche Lenken von Luft auf den Stoff, um die ausgewählten Bereiche zu entfernen, umfasst.

11. Verfahren gemäß einem der Ansprüche 6 bis 9, wobei der Schritt des Entfernens der ausgewählten Bereiche Inkontaktbringen des Stoffs mit Bürsten, um die ausgewählten Bereiche zu entfernen, umfasst.

12. Verfahren gemäß einem der Ansprüche 6 bis 11, wobei der Schritt des Anwendens von Wärme und Druck Inkontaktbringen einer Prägewalze mit einer erwärmten Ambosswalze oder mit einem Ultraschallamboss umfasst.

13. Prägewalze zur Herstellung eines mit Öffnungen versehenen Vliesstoffs, umfassend einen zylindrischen Körper und eine Vielzahl von erhöhten Prägungen an vorbestimmten beabstandeten Stellen an der zylindrischen Oberfläche des Körpers, wobei die erhöhten Prägungen eine erhöhte Stegoberfläche zum Inkontaktbringen mit dem Gewebe, die sich entlang eines geschlossenen Wegs entlang der Peripherie der erhöhten Prägung erstreckt, und eine vertiefte Oberfläche, die von der erhöhten Stegoberfläche umgeben ist, umfassen und wobei die erhöhte Stegoberfläche einen Oberflächenbereich von zwischen 2% und 20% des Bereichs, der von der erhöhten Stegoberfläche umgeben ist, hat, wobei die Prägungen so konzipiert sind, dass sie Stanzabfälle zurücklassen, die lösbar an einigen der Öffnungen befestigt sind, und dass sie einen Rand aus verschmolzener thermoplastischer Faser, der sich entlang der Peripherie der Stanzabfälle erstreckt, umfassen.

14. Walze gemäß Anspruch 13, wobei die Prägungen auf der Walze in einer solchen Dichte vorliegen, dass die erhöhte Stegoberfläche und die umgebene vertiefte Oberfläche wenigstens 10% des Oberflächenbereichs der zylindrischen Oberfläche bilden.

15. Walze gemäß Anspruch 13 oder 14, wobei die erhöhte Stegoberfläche 2 bis 10 Prozent des Oberflächenbereichs des Bereichs, der von der erhöhten Stegoberfläche umgeben ist, bildet.

16. Walze gemäß Anspruch 13, 14 oder 15, wobei die erhöhte Stegoberfläche eine Breite von 10 bis 30 Prozent der maximalen Breite der erhöhten Prägung hat.

17. Walze gemäß einem der Ansprüche 13 bis 16, wobei die erhöhten Prägungen eine kreisförmige oder ovale Konfiguration haben.

## Revendications

1. Etoffe non tissée composée de fibres thermoplastiques liées les unes aux autres en une multiplicité de sites de liaison pour former une bande non tissée solide et cohérente, et une pluralité d'ouvertures formées dans l'étoffe non tissée par retrait de parties sélectionnées de la bande non tissée, les ouvertures formant une région ouverte d'au moins 10 pour cent de l'aire de l'étoffe, l'étoffe incluant une découpe perforée formée sur la partie retirée de la bande non tissée fixée de façon amovible à au moins certaines des ouvertures, une marge de fibre thermoplastique fondue s'étendant le long de la périphérie de la découpe perforée.

2. Etoffe selon la revendication 1, incluant une marge de fibre thérapeutique fondue s'étendant le long de la périphérie des ouvertures.

3. Etoffe selon l'une quelconque des revendications précédentes, dans laquelle l'étoffe non tissée est choisie dans le groupe constitué par une étoffe non tissée à liaison thermique cardée comprenant des fibres discontinues thermoplastiques, une bande non tissée air-laid comprenant des fibres discontinues thermoplastiques, et une étoffe non tissée filée-liée composée de filaments continus de polymère thermoplastique.

4. Etoffe selon l'une quelconque des revendications précédentes, dans laquelle l'étoffe n'est pas étirée.

5. Etoffe non tissée filée-liée composée de filaments thermoplastiques continus agencés de façon aléatoire et liés les uns aux autres en une multiplicité de sites de liaison pour former une bande non tissée filée-liée solide et cohérente, et une pluralité d'ouvertures formées dans l'étoffe non tissée par retrait de parties sélectionnées de la bande non tissée, les ouvertures formant une région ouverte d'au moins 10 pour cent de l'aire de l'étoffe, l'étoffe non tissée filée-liée incluant une découpe perforée formée à partir de la partie retirée de bande non tissée filée-liée fixée de façon amovible à au moins certaines des ouvertures, une marge de fibre thermoplastique fondue s'étendant le long de la périphérie de la découpe perforée.

6. Procédé de fabrication d'une étoffe non tissée à ouvertures comprenant les étapes consistant à :
- diriger une étoffe non tissée composée de fibres thermoplastiques le long d'un trajet de déplacement prédéterminé dans et à travers un poste de gaufrage ;
- mettre en contact l'étoffe non tissée au niveau du poste de gaufrage avec un rouleau de gaufrage ayant une surface à motif prédéterminée ;
- appliquer de la chaleur et une pression à l'étoffe non tissée avec la surface à motif pour faire fondre thermiquement les fibres thermoplastiques le long d'une pluralité de trajets fermés définissant des régions sélectionnées de la surface de l'étoffe dans lesquelles des ouvertures doivent être formées, formant des découpes perforées qui sont attachées de façon amovible à certaines des ouvertures, et formant une marge de fibres thermoplastiques fondues s'étendant autour de la périphérie des découpes perforées ; et
- retirer lesdites régions sélectionnées de l'étoffe du restant de l'étoffe.

7. Procédé selon la revendication 6, dans lequel les régions sélectionnées constituent au moins 10 pour cent de l'aire de l'étoffe.

8. Procédé selon la revendication 6, dans lequel la pluralité de trajets fermés de fibres thermiquement fondues forme des régions gaufrées qui ne constituent pas plus de 10 pour cent de l'aire ce l'étoffe et entourent des régions de l'étoffe non tissée dans lesquelles les fibres thermoplastiques ne sont ni fondues, ni gaufrées.

9. Procédé selon la revendication 8, dans lequel la pluralité de trajets fermés de fibres thermiquement fondues présente une aire comprise entre 2 % et 20 % de l'aire circonscrite par les trajets fermés.

10. Procédé selon l'une quelconque des revendications 6 à 9, dans lequel l'étape consistant à retirer lesdites régions sélectionnées comprend le fait de diriger de l'air sur le tissu pour retirer lesdites régions sélectionnées.

11. Procédé selon l'une quelconque des revendications 6 à 9, dans lequel l'étape consistant à retirer lesdites régions sélectionnées comprend le fait de mettre en contact l'étoffe avec des balais pour retirer lesdites régions sélectionnées.

12. Procédé selon l'une quelconque des revendications 6 à 11, dans lequel l'étape consistant à appliquer de la chaleur et une pression comprend le fait de mettre en contact le rouleau de gaufrage avec un rouleau enclume chauffé ou avec une enclume à ultrasons.

13. Rouleau de gaufrage permettant de produire une étoffe non tissée à ouvertures comprenant un corps cylindrique et une pluralité de foulages surélevés à des emplacements espacés prédéterminés sur la surface cylindrique du corps, lesdits foulages surélevés incluant une surface d'appui surélevée destinée à venir au contact de l'étoffe s'étendant le long d'un trajet fermé le long de la périphérie du foulage surélevé, et une surface évidée entourée par la surface d'appui surélevée, et où la surface d'appui surélevée présente une aire comprise entre 2 % et 20 % de la région entourée par la surface d'appui surélevée, les foulages étant conçus pour laisser des découpes perforées qui sont attachées de façon amovible à certaines des ouvertures et pour inclure une marge de fibre thermoplastique fondue s'étendant le long de la périphérie des découpes perforées.

14. Rouleau selon la revendication 13, dans lequel les foulages sont présents sur le rouleau à une densité telle que la surface d'appui surélevée et la surface évidée entourée constituent au moins 10 pour cent de l'aire de la surface cylindrique.

15. Rouleau selon la revendication 13 ou 14, dans lequel la surface d'appui surélevée constitue de 2 à 10 pour cent de l'aire de la région entourée par la surface d'appui surélevée.

16. Rouleau selon la revendication 13, 14 ou 15, dans lequel la surface d'appui surélevée a une largeur de 10 à 30 pour cent de la largeur maximale du foulage surélevé.

17. Rouleau selon l'une quelconque des revendications 13 à 16, dans lequel les foulages surélevés ont une configuration circulaire ou ovale.
